

# United States Patent Office

2,762,723

Patented Sept. 11, 1956

1

2,762,723

## PROCESSES OF CHEMICAL NICKEL PLATING AND BATHS THEREFOR

Paul Talmey, Barrington, Ill., and Gregoire Gutzeit, Highland, Ind., assignors to General American Transportation Corporation, Chicago, Ill., a corporation of New York

No Drawing. Application June 3, 1953,  
Serial No. 359,428

27 Claims. (Cl. 117—130)

The present invention relates to improved processes of 15 chemical nickel plating of catalytic materials employing baths of the nickel cation-hypophosphite anion type containing stabilizing agents.

The chemical nickel plating of acatalytic material employing an aqueous bath of the nickel cation-hypophosphite anion type is based upon the catalytic reduction of nickel cations to metallic nickel and the corresponding oxidation of hypophosphite anions to phosphite anions with the evolution of hydrogen gas at the catalytic surface. The reactions take place when the body of catalytic 20 material is immersed in the plating bath, and the exterior surface of the body of catalytic material is coated with nickel. The following elements are catalytic for the oxidation of hypophosphite and thus may be directly nickel-plated: iron, cobalt, nickel, ruthenium, rhodium, palladium, osmium, iridium and platinum. The following elements are examples of materials which may be nickel-plated by virtue of the initial displacement deposition of nickel thereon either directly or through a galvanic effect: copper, silver, gold, beryllium, germanium, aluminum, carbon, vanadium, molybdenum, tungsten, chromium, selenium, titanium and uranium. The following elements are examples of non-catalytic materials which ordinarily may not be nickel-plated: bismuth, cadmium, tin, lead and zinc. The activity of the catalytic materials varies considerably; and the following elements are particularly good catalysts in the chemical nickel plating bath: iron, cobalt, nickel and palladium. The chemical nickel plating process is autocatalytic since both the original surface of the body being plated and the nickel metal that is deposited on the surface thereof are both catalytic; and the reduction of the nickel cations to metallic nickel in the plating bath proceeds until all of the nickel cations have been reduced to metallic nickel, in the presence of an excess of hypophosphite anions, or until all of the hypophosphite anions have been oxidized to phosphite anions, in the presence of an excess of nickel cations. Actually the reactions are slowed-down rather rapidly as time proceeds because the anions, as contrasted with the cations, of the nickel salt that is dissolved in the plating bath combine with the hydrogen cations to form an acid, which, in turn, lowers the pH of the bath, and the reducing power of the hypophosphite anions is decreased as the pH value of the bath decreases. Moreover, there is a tendency for the early formation in the plating bath of a "black precipitate" that comprises a random chemical reduction of the nickel cations. Of course, this formation of the black precipitate comprises a decomposition of the plating bath; and is particularly objectionable in that it causes the nickel deposit to be coarse, rough and frequently porous.

For the dual purposes of increasing the stability of the plating bath (preventing the formation of the black precipitate mentioned), and of increasing the normal plating rate of the bath, various baths of the present type have been suggested employing different additives or agents that serve either as buffers or as exaltants. For exam-

2

ple, in the copending application of Gregoire Gutzeit and Abraham Krieg, Serial No. 194,656, filed November 8, 1950, now Patent No. 2,658,841, granted November 10, 1953, there is disclosed a chemical nickel plating bath of the nickel cation-hypophosphite anion type that contains as an additive a buffer in the form of a soluble salt of an organic acid, and specifically sodium acetate; and in the copending application of Gregoire Gutzeit and Ernest J. Ramirez, Serial No. 204,424, filed January 4, 1951, now Patent No. 2,658,842, granted November 10, 1953, there is disclosed a chemical nickel plating bath of the nickel cation-hypophosphite anion type that contains as an additive an exaltant in the form of a soluble salt of a simple short-chain saturated aliphatic dicarboxylic acid, and specifically sodium succinate. A typical chemical nickel plating bath of the character of that disclosed in the Gutzeit and Krieg application essentially comprises an aqueous acid solution of a nickel salt and a hypophosphite and a buffer in the form of an alkaline acetate, the initial pH of the bath being within the approximate range 4.5 to 5.6, the ratio between nickel ions and hypophosphite ions in the bath being between 0.25 and 0.60, the absolute concentrations of hypophosphite ions in the bath being between 0.15 and 0.35 mole/liter, and the absolute concentrations of acetate ions in the bath being approximately 0.120 mole/liter. A typical chemical nickel plating bath of the character of that disclosed in the Gutzeit and Ramirez application essentially comprises an aqueous acid solution of a nickel salt and a hypophosphite and an exaltant in the form of a salt of succinic acid, the initial pH of the bath being within the approximate range 4.3 to 6.8, the ratio between nickel ions and hypophosphite ions in the bath being between 0.25 and 1.60, the absolute concentration of hypophosphite ions in the bath being between 0.15 and 1.20 mole/liter, and the absolute concentration of succinate ions in the bath being at least 0.05 mole/liter.

In carrying out the chemical nickel plating process on a commercial scale employing a plating bath of the types mentioned, there may be utilized a continuous system of the character of that disclosed in the copending application of Paul Talmey and William J. Crehan, Serial No. 222,222, filed April 21, 1951, now Patent No. 2,658,839, granted November 10, 1953; which system involves periodic or continuous regeneration of the plating bath by the addition thereto of appropriate ingredients for the purpose of maintaining substantially constant the composition of the bath.

In carrying out the chemical nickel plating process, particularly in a continuous system of the character mentioned, it has been discovered that an initially stable plating bath becomes unstable after some use, and notwithstanding the content of the buffer, or the exaltant, or both; whereby the plating bath decomposes with the formation of the previously-mentioned black precipitates. (The first visible manifestation in the plating bath of random reduction of the nickel cations) starts at the surfaces of suspensoids (solid particles of dust, microcrystalline precipitate of ferric hypophosphite, nickel phosphite, etc.) present in the plating bath; and the presence of these suspensoids in the plating bath is evidenced by the observation of Tyndall beams when a shaft of light is passed through the clear filtered plating bath, even when freshly prepared.

The present invention is predicated upon the discovery that plating baths of the nickel cation-hypophosphite anion types mentioned may be stabilized to a high degree, without material depression of the plating rates thereof; by the further addition thereto of a trace amount of certain water-soluble additives of dipolar molecular character; the dipolar molecules being water-soluble in

the true sense that a molecular solution is produced, as distinguished from a colloidal solution. In the bath, the cation of the dipolar molecule is readily dissociated and the anion of the dipolar molecule forms with the element of the suspensoid a water-insoluble product that is hydrophobic or water-repellent; the terms "water-repellent" and "hydrophobic" being taken in the broadest sense, indicating an induced surface condition that will repel anions and dipoles of negative character. Thus the additive of dipolar molecular form is of the hydrophobic film-forming class and may take a variety of forms including the sulfhydric compounds, since these compounds have at least one functional group with affinity for metals and a hydrophobic radical characterized by forming oriented water-repellent coatings on metal surfaces.

In accordance with one form of the invention, a trace amount of sulfide ions (if necessary) and a trace amount of a "stabilizing agent" in the form of a "sulfide ion controller" are added to the bath; and specifically it has been discovered that plating baths of the character mentioned are stabilized by the presence therein of extremely small amounts of sulfide ions (S''), which hydrolyze, in the presence of water, to sulfhydric ions (SH'). In larger quantities sulfide ions added to the plating bath, for example as H<sub>2</sub>S, (as well as other ions, such as CN', Pb . . . , Bi . . . , Sn . . . , etc.) are a catalytic poison, and will considerably reduce the plating rate, or stop plating altogether. However, at the proper level, sulfide ions prevent random decomposition of the plating bath and the formation of the black precipitate mentioned; the minimum quantity of sulfide ions in the plating bath to achieve stability being approximately 10 parts per 1,000,000,000 parts of the plating bath by weight.

It is believed that the sulfide ions selectively attach themselves to the suspensoids in the plating bath thereby preventing the suspensoids from serving as nuclei for the random decomposition of the plating bath and the formation of the objectionable black precipitate. Specifically, the sulfide ions seem to be absorbed in an oriented manner upon the surfaces of the suspensoids giving them a hydrophobic (water repellent), which may account for the protective action in inhibiting the formation of the black precipitate. It is not necessary to have a continuous film upon the surfaces of the suspensoids, as it is sufficient that the "active centers" be shielded. This mechanism is considered to be the most likely, as it is well-known that ions or dipoles are absorbed on the surfaces of solids due to localized attractive forces (free valency links), and that these same ions or dipoles repel each other due to their identical electric charges. Thus the packing of these ions or dipoles on a section of surface is a function of the radius of curvature of the surface, so that the smaller the radius of curvature the stronger the bond and the closer the packing. Accordingly, since the radii of the suspensoids are very small, the surfaces thereof will be preferentially and more densely covered than the relatively flat surfaces of any large body to be plated. Consequently the sulfide ions selectively attach themselves first to the suspensoids, thereby preventing their objectionable effect as nuclei for the random decomposition of the plating bath, as explained above. Moreover, the amount of the sulfide ions present should be limited so as not to have an inhibiting effect on the surface of the object being plated.

Sulfur (as such, or as inorganic, respectively organic sulfides) is generally present in very small amounts (of the order of parts per 1,000,000,000) in water and in the chemicals ordinarily used to prepare the plating bath. Elemental sulfur (particularly in a reducing medium) hydrolyzes to hydrogen sulfide; and any other soluble sulfide present in the acid plating bath will also bring about the formation of hydrogen sulfide which is volatile at elevated temperatures and thus escapes from the plating bath. As a result of this loss of sulfide ions, by boil-

ing off of the hydrogen sulfide, the plating bath becomes unstable after a short time interval, as previously noted. Wherever sulfide ions are not fortuitously present in the plating bath, they should be added, preferably as lead sulfide.

It is thought that the addition of traces of sulfide ion controllers that continuously release sulfide ions in controlled amounts in the quantities previously mentioned achieves the stabilization of the plating bath; and it is believed that this is the mechanism of the stabilization. Of course, the cations of the sulfide ion controller must not comprise catalytic poisons in the particular range where they are being used for stabilization; nor should they be themselves catalysts for the oxidation of hypophosphite to phosphite. For practical purposes the S'' ion (respectively SH' ion) can be controlled continuously by two broad classes of compounds:

(1) Inorganic sulfides that are stable and practically insoluble in the plating bath under plating conditions; i. e., in an aqueous acid solution having a pH above 2.5, and particularly in the range from 3.0 to 5.5, and at temperatures above 90° C., provided the cation bound to the sulfur is not a catalyst for the oxidation of hypophosphite; in other words, that it does not belong to group VIII of the periodic system.

(2) Organic and inorganic thio-compounds that are water-soluble and soluble under plating conditions in the plating bath, and which hydrolyze with respect to their sulfur at a rate such that a concentration of at least 10 p. p. b. (parts per billion) of liberated S'' is continuously maintained in the aqueous plating bath.

Insofar as the first class is concerned, it is not necessary to supply the metallic sulfides as such, as there appears to be usually enough sulfur or sulfide ions present in the bath as impurities. It is sufficient, therefore, merely to add traces of elements whose cations form sulfides that are stable and practically insoluble under plating conditions in the aqueous acid plating bath; and an excess of these cations should be avoided as most of them are catalytic poisons. The elements that form sulfide ion controllers and thereby achieve stabilization are: lead, copper, bismuth, tin, selenium, tellurium, tungsten, thorium, titanium, zinc, manganese and rhenium.

Insofar as the second class is concerned, the organic and inorganic thio-compounds are active to achieve stabilization; typical examples are soluble inorganic thiosulfates, thio-cyanate, xanthates, "Aerofloats," thio-acids, thioamines (such as thiocabanilide or thiourea), organic sulfides, etc.; which organic chemicals have a very low dissociation constant (K) relative to their sulfur atoms.

Also in connection with the first class, it is noted that certain of the stabilizing agents increase the normal plating rate of the plating bath in addition to achieving stability; i. e., lead, tin and manganese; while other of these stabilizing agents improve the appearance of the plated article with reference to brightness in addition to achieving stability; i. e., selenium and tellurium.

In view of the foregoing, it is the primary object of the present invention to provide an improved nickel plating process of the character described in which the reactions involved are carried out more efficiently and under more stable conditions than heretofore, thereby rendering the process more desirable from a commercial standpoint.

Another object of the invention is to provide an improved nickel plating process of the character described, that employs a plating bath of the nickel cation-hypophosphite anion type containing as a stabilizing agent an additive of dipolar molecular character.

Another object of the invention is to provide an improved nickel plating process of the character described, that employs a plating bath of the nickel cation-hypophosphite anion type containing as a stabilizing agent a sulfide ion controller.

A further object of the invention is to provide an im-

proved nickel plating process of the character described that comprises a plating bath of the nickel cation-hypophosphite anion type containing as a stabilizing agent organic sulfhydric compounds.

A further object of the invention is to provide an improved nickel plating process of the character described, that employs a plating bath of the type mentioned containing a stabilizing agent that increases the normal plating rate thereof.

A further object of the invention is to provide an improved nickel plating process of the character described that employs a plating bath of the type mentioned containing a stabilizing agent that effects brightening of the nickel deposit.

A still further object of the invention is to provide an improved nickel plating bath of the nickel cation-hypophosphite anion type containing as a stabilizing agent a sulfide ion controller.

These and other objects and advantages of the invention pertain to the particular arrangement of the steps of the method and of the composition of the plating bath, and will be understood from the foregoing and following description.

In accordance with the process of the present invention, the article to be nickel-plated and normally formed of a catalytic material, is properly prepared by mechanically cleaning, degreasing and light pickling, substantially in accordance with standard practices in electroplating processes. For example, in the nickel plating of a steel object, it is customary mechanically to clean the rust and mill scale from the object, to degrease the object, and then lightly to pickle the object in a suitable acid, such as, hydrochloric acid. The article is then immersed in a suitable volume of the bath containing the proper proportions of nickel cations, hypophosphite anions, buffer or exaltant, and stabilizing agent, the pH of the bath having been, if necessary, adjusted to an optimum value by the addition of an appropriate acid or base, and the bath having been heated to a temperature just below its boiling point, such as 99° C., at atmospheric pressure. Almost immediately hydrogen bubbles are formed on the catalytic surface of the steel object and escape in a steady stream from the bath, while the surface of the steel object is slowly coated with metallic nickel (containing some phosphorus). The reaction is continued until the color of the bath (green at the start) shows the absence of nickel, or until the evolution of hydrogen stops, or until it is determined that the required thickness of the nickel coating has been deposited on the steel object. Of course, the steel object is then removed from the bath and rinsed off with water, and is then ready for use; or the bath may be continuously regenerated, the steel object being removed after the desired thickness of nickel has been deposited thereon.

With respect to the composition of the bath, it essentially comprises an aqueous solution containing nickel cations, hypophosphite anions, a buffer or exaltant, and a stabilizing agent. For example, the nickel cations may be derived from nickel chloride; and the hypophosphite anions may be derived from sodium, potassium, lithium, calcium, magnesium, strontium, barium, etc., hypophosphites, or various combinations thereof. Specifically, a suitable bath may be formed in an exceedingly simple manner by dissolving in a hydrochloric acid-water solution nickel chloride and sodium hypophosphite; and then the buffer or exaltant and the stabilizing agent are added thereto, as explained more fully hereinafter. The desired pH of the bath is established by the eventual introduction thereto of additional hydrochloric acid and is appropriately adjusted by the addition thereto of a weak alkali, preferably sodium bicarbonate.

The terms "cation," "anion," and "ion" as employed herein, except where specifically noted, include the total

quantity of the corresponding elements that are present in the plating bath; i. e., both undissociated and dissociated material. In other words, 100% dissociation is assumed when the terms noted are used in connection with molar ratios and concentrations in the plating bath.

The stabilizing effects of the various compounds of the first class were determined from a series of plating tests that were made employing a "standard" test plating bath of the general character of that disclosed in the previously-mentioned Gutzeit and Ramirez application, except that the chemical ingredients were highly purified; this standard test plating bath had a volume of 50 cc. and a temperature between 98° C. and 100° C.; and therein low carbon steel samples were plated that had a surface area of 20 cm.<sup>2</sup> and that had been vapor-degreased, electro-cleaned, and pickled in a 10% HCl solution. The standard test plating bath was produced from a solution containing nickel as nickel hypophosphite (0.09 m. pl.), sodium hypophosphite (0.045 m. pl.), sodium succinate (0.06 m. pl.), sodium chloride (0.18 m. pl.), and enough water to make one liter, the pH having been adjusted to a value of 4.6 with pure HCl, whereby the nickel cation/hypophosphite anion ratio was 0.4. The stabilizing agents were then added to the standard test plating bath by measuring the proper volume from stock solutions containing 1,000 p. p. m. thereof; and the plating rates were measured in gm./cm.<sup>2</sup>% min. In these tests stability is indicated by the time in minutes that elapsed before "black precipitate" was formed; and the appearance of the nickel deposited upon the samples was noted. In describing the appearance of a test sample, the following symbols are employed: B=semi-bright (satin); BB=bright; VB=very bright; S=smooth; SR=slightly rough; R=rough; D=dull; and Sp=spotted.

Two "blank" plating tests were first run employing only the test samples in the standard test plating bath (without the addition of any stabilizing agent), with the following results:

| Duration of Test                               | 10 min. | 60 min.  |
|------------------------------------------------|---------|----------|
| Weight gain, gms.                              | 0.0948  | 0.1003   |
| Plating rate, R <sup>2</sup> X 10 <sup>4</sup> | 4.74    | B-S      |
| Sample appearance                              | B-S     | B-SR     |
| Time to black ppt.                             | None    | 20 mins. |

From the two above blank plating tests, it is apparent that the standard test plating bath is unstable since noticeable decomposition thereof takes place within 20 minutes; and hereafter a plating bath is considered "unstable" in the event it decomposes within a time interval of 60 minutes.

Three stability tests were then run employing the standard test plating bath (without the test samples) at a plating temperature for the purpose of demonstrating the stabilizing effect of lead sulfide. Specifically in the three stability tests lead sulfide in the respective amounts of 52 p. p. b., 43 p. p. b. and zero p. p. b. were added to the standard test plating bath, thereby establishing the respective levels of S" ions therein of 8 p. p. b., 7 p. p. b. and zero p. p. b.; whereby the respective times at which black precipitate formation was observed were: 120 minutes, 16 minutes and 13 minutes. Accordingly, the three stability tests clearly demonstrate that the level at which the S" ion is effective as a stabilizer in the presence of lead is well-defined, the lower threshold of effectiveness being at about 8 p. p. b. and definitely in the range 10 to 100 p. p. b., as will appear more fully hereinafter.

In a series of these plating tests employing the standard test plating bath containing lead as the stabilizing agent, derived from PbCl<sub>2</sub>, the following results were obtained:

## (a) Rate tests—10 minutes

| p. p. m. of Pb <sup>++</sup>  | 0      | 0.01   | 0.04   | 0.07   | 0.10   | 0.20   | 0.40   | 0.50   | 1.0    | 10.0   | 50.0   |
|-------------------------------|--------|--------|--------|--------|--------|--------|--------|--------|--------|--------|--------|
| Wt. gain                      | 0.0919 | 0.0987 | 0.0985 | 0.1037 | 0.0907 | 0.0994 | 0.0986 | 0.0999 | 0.0988 | 0.0554 | 0.0001 |
| Plating Rate, R $\times 10^4$ | 4.59   | 4.94   | 4.93   | 5.18   | 4.54   | 4.97   | 4.93   | 4.49   | 4.69   | 2.77   | D      |
| Sample appearance             | B-S    | BB-S   | BB-S   | BB-S   | BB-S   | BB-S   | BB-S   | BB-S   | BB-S   | BB-S   | none   |
| Time to black ppt.            | none   | none   | none   | none   | none   | none   | none   | none   | none   | none   | none   |

## (b) Stability tests—60 minutes

| p. p. m. of Pb <sup>++</sup> | 0      | 0.01   | 0.04   | 0.07   | 0.10   | 0.20   | 0.4    | 1.0    | 10.0   | 50.0   |
|------------------------------|--------|--------|--------|--------|--------|--------|--------|--------|--------|--------|
| Wt. gain                     | 0.1892 | 0.2110 | 0.2092 | 0.2122 | 0.1896 | 0.1902 | 0.1948 | 0.1907 | 0.1763 | 0.0001 |
| Sample appearance            | B-S    | BB-S   | BB-S   | BB-S   | BB-S   | BB-S   | BB-S   | BB-S   | BB-S   | D      |
| Time to black ppt.           | 16     | 37     | 35     | 43     | stable | stable | stable | stable | stable | stable |

Some of these plating tests employing the standard test plating bath containing lead as the stabilizing agent,

In a series of these plating tests employing the standard test plating bath containing tin as the stabilizing agent, the following results were obtained:

## (a) Rate tests—10 minutes

| p. p. m. of Sn <sup>++</sup>  | 0.1    | 0.5    | 1      | 2      | 10     | 50     | 100    |
|-------------------------------|--------|--------|--------|--------|--------|--------|--------|
| Wt. gain                      | 0.1064 | 0.1072 | 0.0880 | 0.1135 | 0.0998 | 0.0910 | 0.0847 |
| Plating rate, R $\times 10^4$ | 5.32   | 5.36   | 4.40   | 5.68   | 4.99   | 4.56   | 4.26   |
| Sample appear                 | B-S    | BB-S   | BB-S   | B-S    | B-S    | B-S    | B-S    |
| Time to black ppt.            | none   | none   | none   | none   | none   | none   | none   |

## (b) Stability tests—60 minutes

| p. p. m. of Sn <sup>++</sup> | 0.1    | 0.5    | 1      | 2      | 10     | 50     | 100    |
|------------------------------|--------|--------|--------|--------|--------|--------|--------|
| Wt. gain                     | 0.2189 | 0.2204 | 0.1865 | 0.2220 | 0.1905 | 0.1872 | 0.1776 |
| Sample appear                | B-S    | BB-S   | BB-S   | B-S    | B-S    | B-S    | B-S    |
| Time to black ppt.           | 40     | 40     | 25     | stable | stable | stable | stable |

derived from Pb(NO<sub>3</sub>)<sub>2</sub>, were repeated; and the following results were obtained:

| p. p. m. of Pb <sup>++</sup>  | 1.0    | 2.0    | 1.0    | 2.0    |
|-------------------------------|--------|--------|--------|--------|
| Duration of Test, mins.       | 10     | 10     | 60     | 60     |
| Wt. gain                      | 0.0927 | 0.0771 | 0.1719 | 0.1596 |
| Plating rate, R $\times 10^4$ | 4.68   | 3.85   | BB-S   | BB-S   |
| Sample Appearance             | BB-S   | stable | BB-S   | stable |
| Time to black ppt.            | none   | none   | none   | none   |

40 In view of the foregoing plating test employing in the standard test plating bath tin as the stabilizing agent, the stabilizing range is about 2.0 to 50.0 p. p. m., the plating rate being increased at 2.0 p. p. m.

In a series of these plating tests employing the standard test plating bath containing manganese as the stabilizing agent the following results were obtained:

45

## (a) Rate tests—10 minutes

| p. p. m. of Mn <sup>++</sup>  | 0      | 1      | 2      | 3.3    | 5      | 10     | 25     | 50     |
|-------------------------------|--------|--------|--------|--------|--------|--------|--------|--------|
| Wt. gain                      | 0.0948 | 0.9068 | 0.1046 | 0.1050 | 0.0792 | 0.0812 | 0.0937 | 0.0969 |
| Plating rate, R $\times 10^4$ | 4.74   | 4.84   | 5.23   | 5.25   | 3.96   | 4.06   | 4.94   | 4.84   |
| Sample appear                 | B-S    | BB-S   | BB-S   | BB-S   | BB-S   | BB-S   | B-R    | B-R    |
| Time to black ppt.            | none   | none   | none   | none   | none   | none   | none   | none   |

## (b) Stability tests—60 minutes

| p. p. m. of Mn <sup>++</sup> | 0      | 1      | 2      | 3.3    | 5      | 10     |
|------------------------------|--------|--------|--------|--------|--------|--------|
| Wt. gain                     | 0.1903 | 0.1933 | 0.1952 | 0.1943 | 0.1864 | 0.1921 |
| Sample appear                | B-SR   | B-SR   | BB-S   | BB-S   | B-SR   | B-SR   |
| Time to black ppt.           | 20     | 30     | stable | stable | 40     | 40     |

In view of the foregoing plating tests employing in the standard test plating bath lead as the stabilizing agent, it will be observed that about 0.1 p. p. m. of Pb<sup>++</sup> is required in order to obtain a stable bath; and at about 10 p. p. m. of Pb<sup>++</sup>, the plating rate starts to decline. Finally, the peculiar phenomenon is exhibited that the trace of lead between 0.01 and 1.0 p. p. m. actually enhances or exalts the plating rate, a maximum exaltation appearing between 0.01 and 0.07 p. p. m.

70 In view of the foregoing plating tests employing in the standard test plating bath manganese as the stabilizing agent, it will be observed that stabilization is obtained at concentrations between 1.0 and 4.0 p. p. m. and that the plating rate is somewhat enhanced.

In a series of these plating tests employing the standard test plating bath containing selenium as the stabilizing agent, the following results were obtained:

75

## (a) Rate tests—10 minutes

| p. p. m. of $\text{SeO}^{2-}$        | 1      | 2      | 5      |
|--------------------------------------|--------|--------|--------|
| Wt. gain                             | 0.0750 | 0.0778 | 0.0034 |
| Plating rate, $\text{R} \times 10^4$ | 3.75   | 3.65   | 0.17   |
| Sample appearance                    | BB-S   | BB-S   | BB-S   |
| Time to black ppt.                   | none   | none   | none   |

## (b) Stability tests—60 minutes

| p. p. m. of $\text{SeO}^{2-}$ | 1      | 2      | 5      |
|-------------------------------|--------|--------|--------|
| Wt. gain                      | 0.1969 | 0.1526 | 0.1391 |
| Sample appearance             | BB-S   | BB-S   | BB-S   |
| Time to black ppt.            | 25     | 45     | stable |

In view of the foregoing plating tests employing in the standard test plating bath selenium as the stabilizing agent, it will be observed that at about 5.0 p. p. m. of selenium the bath is stabilized; and in passing, it is noted that identical results were obtained with the selenite and selenate anions with brightening of the nickel deposit.

In a series of these plating tests employing the standard test plating bath containing tellurium as the stabilizing agent the following results were obtained:

## (a) Rate tests—10 minutes

| p. p. m. of $\text{Te}^{4-}$         | 0.1    | 1      | 5      | 10     |
|--------------------------------------|--------|--------|--------|--------|
| Wt. gain                             | 0.0666 | 0.0468 | 0.0468 | 0.0431 |
| Plating rate, $\text{R} \times 10^4$ | 3.33   | 2.34   | 2.34   | 2.15   |
| Sample appearance                    | B-S    | BB-S   | BB-S   | BB-S   |
| Time to black ppt.                   | none   | none   | none   | none   |

## (b) Stability tests—60 minutes

| p. p. m. of $\text{Te}^{4-}$ | 0.1    | 1      | 5      | 10     |
|------------------------------|--------|--------|--------|--------|
| Wt. gain                     | 0.1495 | 0.1285 | 0.1218 | 0.1128 |
| Sample appearance            | B-S    | BB-S   | B-S    | B-S    |
| Time to black ppt.           | stable | stable | stable | stable |

| p. p. m. of $\text{TeO}_3^{2-}$ | 1      | 5      | 10     | 160    |
|---------------------------------|--------|--------|--------|--------|
| Wt. gain                        | 0.1324 | 0.1341 | 0.1388 | 0.1900 |
| Sample appearance               | BB-S   | VB-S   | VB-S   | BB-S   |
| Time to black ppt.              | stable | stable | stable | stable |

In view of the foregoing plating tests employing in the standard test plating bath tellurium as the stabilizing agent, it will be observed that stabilization is obtained at about 0.1 p. p. m. and that very bright relatively soft nickel deposits are obtained. In passing, it is noted that the tellurate anion gives results identical to those obtained with the tellurite anion, as probably the  $\text{TeO}_4^{2-}$

anion is reduced to the  $\text{TeO}_3^{2-}$  anion by the hypophosphite.

In a series of these plating tests employing the standard test plating bath containing bismuth as the stabilizing agent, the following results were obtained:

## (a) Rate tests—10 minutes

| p. p. m. of $\text{Bi}^{3+}$         | 0.5    | 1      | 5      | 10     |
|--------------------------------------|--------|--------|--------|--------|
| Wt. gain                             | 0.0654 | 0.0832 | 0.0610 | 0.0708 |
| Plating rate, $\text{R} \times 10^4$ | 3.27   | 4.16   | 3.05   | 3.54   |

## (b) Stability tests—60 minutes

| p. p. m. of $\text{Bi}^{3+}$ | 0.5    | 1      | 5      | 10     |
|------------------------------|--------|--------|--------|--------|
| Wt. gain                     | 0.1491 | 0.1524 | 0.1514 | 0.1442 |
| Sample appearance            | BB-S   | BB-S   | BB-S   | BB-S   |
| Time to black ppt.           | 20     | stable | stable | 30     |

In view of the foregoing plating tests employing in the standard test plating bath bismuth as the stabilizing agent, it will be observed that stabilization occurs at concentrations between 1.0 and 5.0 p. p. m., the maximum rate being at about 1.0 p. p. m.

In a series of these plating tests employing the standard test plating bath containing copper as the stabilizing agent, the following results were obtained:

## (a) Rate tests—10 minutes

| p. p. m. of $\text{Cu}^{2+}$ | 1      | 22.1   |
|------------------------------|--------|--------|
| Wt. gain                     | 0.0700 | 0.1059 |
| Plating rate                 | 3.53   | 5.29   |

| p. p. m. of $\text{Cu}^{2+}$ | 5      | 10     | 22.1   | 50     |
|------------------------------|--------|--------|--------|--------|
| Wt. gain                     | 0.1222 | 0.1271 | 0.1264 | 0.1310 |
| Sample appearance            | B-SR   | BB-S   | BB-S   | B-S    |
| Time to black ppt.           | 29     | 42     | stable | stable |

Some of these plating tests employing the standard test plating bath containing cuprous cation ( $\text{Cu}^{+}$ ) were repeated; and the following results were obtained:

| p. p. m. of $\text{Cu}^{+}$ | 5      | 10     | 20     | 50     |
|-----------------------------|--------|--------|--------|--------|
| Wt. gain                    | 0.1282 | 0.1216 | 0.1123 | 0.08-6 |
| Sample appearance           | B-S    | B-S    | B-S    | BB2S   |
| Time to black ppt.          | 35     | stable | stable | stable |

In view of the foregoing plating tests employing in the standard test plating bath copper as the stabilizing agent, it will be observed that the cupric cation ( $\text{Cu}^{2+}$ ) is stabilizing within the range 20 to 50 p. p. m.; while the cuprous cation ( $\text{Cu}^{+}$ ) is stabilizing above 10 p. p. m.

In a series of these plating tests employing the standard test plating bath containing rhenium as the stabilizing agent, the following results were obtained:

## (a) Rate tests—10 minutes

| p. p. m. of $\text{ReO}_4^-$         | 1      | 5      | 10     | 25     |
|--------------------------------------|--------|--------|--------|--------|
| Wt. gain                             | 0.0860 | 0.0907 | 0.0848 | 0.0726 |
| Plating rate, $\text{R} \times 10^4$ | 4.30   | 4.54   | 4.24   | 3.63   |

## 11

## (b) Stability tests—60 minutes

| p. p. m. of $\text{ReO}_4^-$ | 1      | 5      | 10     | 25     |
|------------------------------|--------|--------|--------|--------|
| Wt. gain                     | 0.1528 | 0.1526 | 0.1556 | 0.1527 |
| Sample appearance            | B-S    | B-S    | B-SR   | B-SR   |
| Time to black ppt.           | 20     | 20     | 40     | 30     |

Some of these plating tests employing the standard test plating bath containing  $\text{Re}^{4+}$  cation were repeated, and the following results were obtained:

| p. p. m. of $\text{Re}^{4+}$ | 1      | 5      | 10     |
|------------------------------|--------|--------|--------|
| Wt. gain                     | 0.1173 | 0.0996 | 0.0502 |
| Sample appearance            | B-S    | B-S    | B-S    |
| Time to black ppt.           | 28     | stable | stable |

In view of the foregoing plating tests employing in the standard test plating bath rhenium as the stabilizing agent, it will be observed that the perrhenate cations  $\text{ReO}_4^+$  is not stabilizing, whereas the  $\text{R}^{4+}$  cation is stabilizing at a concentration of about 5 p. p. m.

In a series of these plating tests employing the standard test plating bath containing thorium as the stabilizing agent, the following results were obtained:

## Stability tests—60 minutes

| p. p. m. of Th     | 1      | 5      | 10     |
|--------------------|--------|--------|--------|
| Wt. gain           | 0.1301 | 0.1213 | 0.1233 |
| Sample appearance  | B-S    | B-S    | B-S    |
| Time to black ppt. | stable | stable | 40     |

In view of the foregoing plating tests employing in the standard test bath thorium as the stabilizing agent, it will be observed that the peculiar condition is encountered that stabilization is obtained in the range 1 to 5 p. p. m., but not at higher concentrations at about 10.0 p. p. m., the plating rate being somewhat reduced.

In a series of these plating tests employing the standard test plating bath containing titanium as the stabilizing agent, the following results were obtained:

## Stability tests—60 minutes

| p. p. m. of Ti     | 1        | 5        | 10         |
|--------------------|----------|----------|------------|
| Wt. gain           | 0.1033   | 0.0048   | no plating |
| Sample appearance  | D-stable | D-stable | D-stable   |
| Time to black ppt. |          |          |            |
| p. p. m. of Ti     | 1        | 5        | 10         |
| Wt. gain           | 0.1309   | 0.1060   | 0.0803     |
| Sample appearance  | B-S      | B-S      | B-S        |
| Time to black ppt. | 13       | stable   | stable     |

In view of the foregoing plating tests employing in the standard test plating bath titanium as the stabilizing agent, it will be observed that the  $\text{Ti}^{4+}$  cation produces stabilization at about 1.0 p. p. m. with dull plating and considerable reduction in the plating rate; but that the  $\text{Ti}^{4+}$  cation is stabilizing at about 5.0 p. p. m. with a low plating rate.

In a series of these plating tests employing the standard test plating bath containing tungsten as the stabilizing agent, the following results were obtained:

## Stability tests—60 minutes

| p. p. m. of $\text{WO}_3^{4-}$ | 1      | 5      | 10     |
|--------------------------------|--------|--------|--------|
| Wt. gain                       | 0.1286 | 0.1350 | 0.1336 |
| Sample appearance              | B-S    | B-S    | B-S    |
| Time to black ppt.             | 17     | stable | 35     |

## 12

In view of the foregoing plating tests employing in the standard test plating bath tungsten as the stabilizing agent, it will be observed that stabilization is obtained at a concentration rather sharply defined at 5.0 p. p. m., the plating rate being somewhat reduced.

In a series of these plating tests employing the standard test plating bath containing zinc as the stabilizing agent, the following results were obtained:

## Stability tests—60 minutes

| p. p. m. Zn <sup>2+</sup> | 1      | 5      | 10     | 20     | 30     | 50     |
|---------------------------|--------|--------|--------|--------|--------|--------|
| Wt. gain                  | 0.1303 | 0.1321 | 0.1318 | 0.1259 | 0.1100 | 0.1093 |
| Sample appearance         | B-S    | B-S    | B-S    | B-S    | D-S    | D-S    |
| Time to black ppt.        | 27     | 56     | 41     | stable | stable | stable |

In view of the foregoing plating tests employing in the standard test bath zinc as the stabilizing agent, it will be observed that stabilization is obtained at about 20.0 p. p. m. and above, the plating rate being somewhat depressed.

It is noted that the above-mentioned metallic cations all form sulfides that are both substantially insoluble in the plating bath at a pH above 2.5 and stable at the plating temperature (90° C. and above). These elements all belong to the recognized qualitative analytical groups I and II, and specifically to subgroups Ia, Ib, IIb and IIc. As a matter of fact, if both the metals that are catalysts for the oxidation of hypophosphite to phosphite and that form unstable sulfides in boiling water or at pH values above 2.5 are excluded, it can be stated that the inorganic stabilizing elements are those of groups I, IIb and IIc.

In a series of these plating tests employing the standard test plating bath using a sulfur-containing molecule (inorganic thio-compounds) as the stabilizing agent, the following results were obtained:

## (a) Rate tests—10 minutes

| p. p. m. of $\text{S}_2\text{O}_3^{2-}$ | 0.5    | 1      | 5      | 10     |
|-----------------------------------------|--------|--------|--------|--------|
| Wt. gain                                | 0.0906 | 0.0926 | 0.0912 | 0.0049 |
| Plating rate, $\text{R} \times 10^4$    | 4.53   | 4.63   | 4.56   | 0.02   |
| Sample appearance                       | D-S    | D-S    | B-S    | D-R    |
| Time to black ppt.                      | none   | none   | none   | none   |

| p. p. m. of $\text{CNS}^-$           | 0.5    | 1      | 5     |
|--------------------------------------|--------|--------|-------|
| Wt. gain                             | 0.1145 | 0.1077 | None  |
| Plating rate, $\text{R} \times 10^4$ | 5.73   | 5.39   | 0.0   |
| Sample appearance                    | B-S    | B-S    | none  |
| Time to black ppt.                   | none   | none   | ----- |

## (b) Stability tests—60 minutes

| p. p. m. of $\text{S}_2\text{O}_3^{2-}$ | 0.5    | 1      | 5      | 10     |
|-----------------------------------------|--------|--------|--------|--------|
| Wt. gain                                | 0.1450 | 0.1458 | 0.1490 | 0.1240 |
| Sample appearance                       | D-S    | D-S    | B-S    | D-R    |
| Time to black ppt.                      | 30     | stable | stable | stable |

| p. p. m. of $\text{CNS}^-$ | 0.5    | 1      |
|----------------------------|--------|--------|
| Wt. gain                   | 0.1742 | 0.1685 |
| Sample appearance          | B-S    | B-S    |
| Time to black ppt.         | stable | stable |

In view of the foregoing plating tests employing in the standard test bath sulfur (inorganic thio-compounds) as the stabilizing agent, it will be observed that the thiosulfate anion stabilizes at concentrations of about 1.0 to 5.0 p. p. m. while the thiocyanate anion stabilizes at concentrations between 0.5 and 1.0 p. p. m.

When the nickel cation concentration in the plating

bath is increased, the amount of stabilizing agent that must be added thereto must be disproportionately increased as indicated by the plating test explained below. In carrying out these tests, a "special" test plating bath was produced from a solution containing nickel as nickel hypophosphite (0.18 m. p. l.), sodium hypophosphite (0.09 m. p. l.), sodium succinate (0.12 m. p. l.), sodium chloride (0.36 m. p. l.), and enough water to make one liter, the pH having been adjusted to a value of 4.63 with pure HCl, whereby the nickel cation/hypophosphite anion ratio was 0.4. This special plating bath had a volume of 50 cc. and a temperature of between 98° C. and 100° C.; and therein low carbon steel samples were plated that had a surface area of 20 cm.<sup>2</sup> that had been vapor-degreased, electro-cleaned and pickled in a 10% HCl solution.

Four "blank" plating tests were first run employing only the test samples in the special test plating bath (without the addition of any stabilizing agent), with the following results:

| Duration of test (minutes)    | 10     | 10     | 60     | 60      |
|-------------------------------|--------|--------|--------|---------|
| Wt. gain, gms.                | 0.0797 | 0.0625 | 0.1376 | 0.2041  |
| Plating rate, R $\times 10^4$ | 3.99   | 3.13   |        |         |
| Sample appearance             | B-R    | B-S    | B-S    | B-R     |
| Time to black ppt.            | 5 min. | none   | 5 min. | 10 min. |

The inconsistencies in these plating tests with regard to the weight gains are due to the formation of black precipitate in the plating baths and the trapping thereof in the nickel deposits upon the samples.

In a series of these plating tests employing the special test plating bath containing lead as the stabilizing agent, the following results were obtained:

(a) Rate tests—10 minutes

| p. p. m. of Pb <sup>+</sup>   | 1      | 5      | 10     | 15     | 20     |
|-------------------------------|--------|--------|--------|--------|--------|
| Wt. gain                      | 0.1111 | 0.0559 | 0.0577 | 0.0544 | 0.0541 |
| Plating rate, R $\times 10^4$ | 5.56   | 2.80   | 2.89   | 2.72   | 2.71   |
| Sample appearance             | B-R    | B-S    | B-S    | B-S    | B-S    |
| Time to black ppt.            | 5 min. | none   | none   | none   | none   |

(b) Stability tests—60 minutes

| p. p. m. of Pb <sup>+</sup> | 1      | 5       | 10      | 15     | 20     |
|-----------------------------|--------|---------|---------|--------|--------|
| Wt. gain                    | 0.1956 | 0.1924  | 0.1965  | 0.2096 | 0.2043 |
| Sample appearance           | B-R    | BB-S    | BB-S    | BB-S   | BB-S   |
| Time to black ppt.          | 5 min. | 30 min. | 40 min. | stable | stable |

By comparison of the plating tests respectively involving the standard test plating bath and the special test plating bath, it will be observed that as little as 0.1 p. p. m. of Pb<sup>+</sup> cation is effective to produce stabilization in the standard test plating bath, whereas 15.0 p. p. m. Pb<sup>+</sup> cation is required to effect stabilization in the special test plating bath. In other words, in order to obtain stabilization in the special test plating bath containing a 2-fold increase of nickel cation, it is necessary to provide a 150-fold increase of Pb<sup>+</sup> cation.

A few of these plating tests employing the special test plating bath containing sulfur (inorganic thio-compound) as the stabilizing agent were repeated with the following results:

(a) Rate tests—10 minutes

| p. p. m. of CNS'              | 1      | 5      | 10     |
|-------------------------------|--------|--------|--------|
| Wt. gain                      | 0.1364 | 0.0025 | 0.0013 |
| Plating rate, R $\times 10^4$ | 6.82   | 0.13   | 0.07   |
| Sample appearance             | BB-S   | B-S    | B-S    |
| Time to black ppt.            | none   | none   | none   |

(b) Stability tests—60 minutes

| p. p. m. of CNS'   | 1       | 5      | 10     |
|--------------------|---------|--------|--------|
| Wt. gain           | 0.2385  | 0.0046 | 0.0038 |
| Sample appearance  | B-S     | D-S    | D-S    |
| Time to black ppt. | 25 min. | stable | stable |

Again it will be observed that while stabilization takes place with 0.5 p. p. m. of CNS' anion in the standard test plating bath more than 1.0 p. p. m. (and less than 5.0 p. p. m.) of CNS' anion is required in the special test plating bath.

The effective minimum amounts of the different ones of these stabilizing agents to achieve stabilization are not only a function of nickel cation concentration in the plating baths, as previously explained, but they also depend upon the particular compositions of the plating baths with reference to other constituents. To illustrate this phenomena three baths "A," "B" and "C" were prepared having the particular composition with respect to other ingredients as follows:

25 Both compositions (for 1 liter aqueous solution):

|                                             | M. p. l. |
|---------------------------------------------|----------|
| A. Nickel as nickel hypophosphite           | 0.09     |
| Sodium hypophosphite                        | 0.045    |
| Sodium chloride                             | 0.18     |
| Sodium succinate                            | 0.06     |
| pH adjusted to 4.60 with pure HCl.          |          |
| B. Nickel as nickel hypophosphite           | 0.09     |
| Sodium hypophosphite                        | 0.045    |
| Sodium chloride                             | 0.18     |
| Amino-acetic acid                           | 0.18     |
| pH adjusted to 4.60 with pure NaOH and HCl. |          |
| C. Nickel as nickel hypophosphite           | 0.09     |
| Sodium hypophosphite                        | 0.045    |
| Sodium chloride                             | 0.18     |
| Malic acid                                  | 0.18     |
| Sodium succinate                            | 0.06     |
| pH adjusted to 4.60 with pure NaOH and HCl. |          |

45 Plating tests were conducted for 60 minutes at about 99° C. on pickled and degreased samples of the character previously mentioned each having a surface area of 20 cm.<sup>2</sup> and the following weight gain figures (gm.) were obtained employing no stabilizing agent and the respective stabilizing agents tellurium, lead, and thiocyanate as indicated below:

| 55 | Bath | Initial pH | No stabilizing agent added | Time to black ppt. in min. |
|----|------|------------|----------------------------|----------------------------|
| A  |      | 4.6        | 0.1892                     | 20                         |
| B  |      | 4.5        | 0.1077                     | 29                         |
| B  |      | 6.5        | 0.2176                     | 22                         |
| B  |      | 8.5        | 0.1597                     | 4                          |
| C  |      | 4.50       | 0.2110                     | 32                         |
| C  |      | 5.50       | 0.2126                     | 15                         |

| 65 | Bath | Initial pH | Time to black ppt. min. | Tellurium—p. p. m. |        |        |        |
|----|------|------------|-------------------------|--------------------|--------|--------|--------|
|    |      |            |                         | 1                  | 5      | 10     | 160    |
| A  |      | 4.6        | None                    | 0.1285             | 0.1218 | 0.1123 | 0.1900 |
| B  |      | 4.5        | None                    | 0.1018             | 0.1037 | 0.1023 |        |
| B  |      | 6.5        | None                    | 0.2614             | 0.2592 | 0.2571 |        |
| B  |      | 8.5        | 20-30                   | 0.2270             | 0.2570 | 0.2755 |        |
| C  |      | 4.50       | None                    | 0.1954             | 0.1828 | 0.1748 |        |
| C  |      | 5.50       | None                    | 0.2296             | 0.2324 | 0.2276 | 0.1824 |

| Bath | Initial pH | Time to black ppt., min. | Lead—p. p. m. |                             |        |        |
|------|------------|--------------------------|---------------|-----------------------------|--------|--------|
|      |            |                          | 0.07          | 1                           | 5      | 10     |
| A    | 4.6        | None                     | 0.2122        | 0.1907                      | 0.0930 | 0.1763 |
| B    | 4.5        | None                     |               | 0.1111                      | 0.0930 | 0.0739 |
| B    | 6.5        | None                     |               | 0.2558                      | 0.2301 | 0.1864 |
| B    | 8.5        | 20-30                    |               | no effect up to 50 p. p. m. |        |        |
| C    | 4.5        | None                     |               | 0.2151                      | 0.2116 | 0.1986 |
| C    | 5.50       | None                     |               | 0.2448                      | 0.2380 | 0.2320 |

| Bath | Initial pH | Time to black ppt., min. | Thiocyanate—p. p. m. |            |        |
|------|------------|--------------------------|----------------------|------------|--------|
|      |            |                          | 1                    | 5          | 10     |
| A    | 4.6        | None                     | 0.1685               | no plating |        |
| B    | 4.5        | None                     | 0.1552               | 0.0016     | 0.0008 |
| B    | 6.5        | None                     | 0.2666               | no plating |        |
| B    | 8.5        | 20-30                    | 0.2908               | no plating |        |
| C    | 4.5        | None                     | 0.2131               | 0.0014     | 0.0010 |
| C    | 5.50       | None                     | 0.2284               | 0.0028     | 0.0006 |

From the above table, it will be observed that in bath "B," at pH 8.5, while Te<sup>+</sup> cation actually increases the plating rate, Pb<sup>+</sup> cation is of no effect within the range set forth. However, in other tests (not reported in detail at this point) it has been demonstrated that Pb<sup>+</sup> cation is effective at 75 p. p. m. (decreased plating rate: 0.1467 gms. gained) and at 100 p. p. m. (increased plating rate: 0.1852 gms. gained).

In passing, it is noted that the stabilizing agents can be introduced into the plating bath by other means than by adding a solution of a soluble salt; i. e., the plating can be performed in the plating bath in the presence of a strip of metallic lead, providing there are enough S<sup>2-</sup> ions in the bath as previously explained.

In the foregoing plating tests, steel samples were used for studying the actions of the stabilizing agents, but the same stabilizing effects have been found to hold true in the plating of other materials such as brass, copper, aluminum, manganese, etc.

As previously pointed out, initially stable plating baths of the character disclosed in the Gutzeit and Krieg application and in the Gutzeit and Ramirez application are sometimes fortuitously obtained by the production of these baths from commercial grades of chemical ingredients by virtue of a content of extraneous sulfur and heavy metals cations (lead, copper, manganese, titanium, etc.) as impurities; however, this result is not obtained when these baths are formed of sufficiently pure chemical ingredients. Moreover the baths even though initially stable due to the fortuitous circumstance mentioned become unstable in use, in continuous plating systems, and particularly in the system disclosed in the Talmey and Crehan application. This rendering unstable of the initially stable plating baths after use is brought about fundamentally by the loss therefrom, by boiling off, of hydrogen sulfide. Thus in order both to obtain initial stability and to insure continued stability of the plating bath in use, the inclusion therein of the stabilizing elements as previously described is highly desirable.

Specifically in carrying out the present method, particularly when a continuous plating operation of the character of that disclosed in the Talmey and Crehan application is employed, it is recommended that the selected stabilizing agent be fed periodically or continuously into the plating bath along with the other regenerating chemicals (particularly the nickel cation and the hypophosphite anion) so as to keep the level thereof substantially constant and at that required, as previously explained; for example, the simplest and safest procedure is to select a stabilizing agent that is known to be active, and unobjectionable with respect to decreasing the plating rate, over a relatively wide range of concentration, such for instance as lead or tin, and to keep the level of concentration thereof within the effective range by the required ad-

dition thereof to the plating bath along with the other regenerating ingredients as noted above.

Turning now to the stabilizing agents of the second class or organic thio-compound type, the sulfhydric flotation collectors have been found to be particularly effective. Specifically the xanthates, of the general formula:



10

Where R is an alkyl group, or a hydroaromatic, respectively an aryl group linked through aliphatic substituents; and M an alkali metal (Na or K), are excellent "sulfide controllers." The most common commercial xanthates (and commercial names) that have been found effective are:

- 15 Potassium ethyl xanthate (Z-3)
- Sodium ethyl xanthate (Z-4)
- Sodium isopropyl xanthate (Z-9)
- Potassium n-butyl xanthate (Z-7)
- Potassium sec-butyl xanthate (Z-8)
- Potassium amyl xanthate (Z-5)
- Pentasol xanthate (Z-6)
- Potassium hexyl xanthate (Z-10)

25

The thiophosphates also belong to the sulfhydric class and are well-known as flotation collectors; they comprise reaction products of phosphorus pentasulfide with various organic compounds such as phenols, alcohols, mercaptans or thioalcohols, amines and nitriles; the products with phenols and alcohols are in common use, known as "Aero-floats" and have the general structural formula:



30 40 wherein R is an alkyl or aryl radical and M an alkali metal or ammonium ion.

Other useful members of the sulfhydric class are mercaptans or thioalcohols; thiocarbanilide (diphenyl thiourea); diphenyl thicarbazide; mercaptobenzothiazole (Flotagen); dithiocarbamates; trithiocarbamates, etc. Also the oxidation products of the above compound (organic sulfides) are effective.

45 50 55 The stabilizing effect of the various compounds of the second class were determined from a series of plating tests that were made employing the standard test plating bath and plating conditions previously described; and plating rates were again measured in gms./cm.<sup>2</sup>/min. In these plating tests the stabilizing agents were added to the standard test plating baths from stock solutions containing 1,000 p. p. m. of the organic molecule.

55 60 In a series of these plating tests employing the standard test plating bath containing potassium ethyl xanthate as the stabilizing agent, the following results were obtained:

60 (a) Rate tests—10 minutes

| p. p. m. of xanthate          | 1      | 5      | 10     | 50     | 250    |
|-------------------------------|--------|--------|--------|--------|--------|
| Wt. gain, gms.                | 0.0953 | 0.0980 | 0.0985 | 0.0910 | 0.0031 |
| Plating rate, R $\times 10^4$ | 4.76   | 4.90   | 4.92   | 4.55   | 0.01   |
| Sample appearance             | B-S    | B-S    | B-S    | D-S    | D-R    |
| Time to black ppt.            | none   | none   | none   | none   | none   |

65 (b) Stability tests—60 minutes

| p. p. m. of xanthate | 1      | 5      | 10     | 50     | 250    |
|----------------------|--------|--------|--------|--------|--------|
| Wt. gain, gms.       | 0.1492 | 0.1480 | 0.1489 | 0.1533 | 0.0031 |
| Sample appearance    | B-S    | B-S    | B-R    | D-S    | D-R    |
| Time to black ppt.   | 45     | stable | stable | stable | stable |

In view of the foregoing plating tests employing in the standard test plating bath potassium ethyl xanthate as the stabilizing agent, it will be observed that stabilization is achieved at 5.0 p. p. m. with a slight increase in the plating rate up to about 10.0 p. p. m. and perhaps to 50.0 p. p. m.

In a series of these plating tests employing the standard test plating bath containing potassium methyl xanthate as the stabilizing agent, the following results were obtained:

(a) Rate tests—10 minutes

| p. p. m. of xanthate          | 0      | 5      | 10     | 25     |
|-------------------------------|--------|--------|--------|--------|
| Wt. gain, gms                 | 0.0566 | 0.0850 | 0.0750 | 0.0890 |
| Plating rate, $R \times 10^4$ | 2.83   | 4.25   | 3.75   | 3.45   |
| pH begin                      | 4.58   | 4.58   | 4.58   | 4.58   |
| pH end                        | 4.00   | 3.81   | 3.89   | 3.95   |
| Sample appearance             | B-S    | B-S    | B-S    | B-S    |
| Time to black ppt             | none   | none   | none   | none   |

(b) Stability tests—60 minutes

| p. p. m. of xanthate | 0      | 1      | 5      | 10     | 25     | 50     |
|----------------------|--------|--------|--------|--------|--------|--------|
| Wt. gain, gms        | 0.1407 | 0.1448 | 0.1477 | 0.1517 | 0.1522 | 0.1540 |
| pH begin             | 4.58   | 4.58   | 4.58   | 4.58   | 4.58   | 4.58   |
| pH end               | 2.72   | 2.63   | 2.66   | 2.64   | 2.65   | 2.70   |
| Sample app           | R      | B      | B      | B      | B      | B      |
| Time to black ppt    | 10     | 10     | 15     | 50     | 55     | stable |

In view of the foregoing plating tests employing in the standard test plating bath potassium methyl xanthate as the stabilizing agent, it will be observed that stabilization is achieved at 50.0 p. p. m. and above.

Comparing the two foregoing groups of plating tests respectively employing in the standard test plating bath potassium ethyl xanthate and potassium methyl xanthate as stabilizing agents, it will be observed that about ten times as much potassium methyl xanthate as potassium ethyl xanthate is required to achieve the same degree of stabilization in the standard test plating bath, thereby indicating that the longer carboxylic chain is clearly functional in the formation of a hydrophobic aliphatic chain product upon the suspensoids.

In a series of these plating tests employing a standard test plating bath containing sodium "Aerofloat" as the stabilizing agent, the following results were obtained:

Stability tests—60 minutes

| p. p. m. sodium "Aerofloat" | 0      | 1      | 5      | 10     | 20     | 30     | 50     | 300        |
|-----------------------------|--------|--------|--------|--------|--------|--------|--------|------------|
| Wt. gain, gms               | 0.1353 | 0.1384 | 0.1415 | 0.1415 | 0.1523 | 0.0060 | 0.0018 | no plating |
| Sample appearance           | B-R    | B-S    | B-S    | B-S    | B-S    | D      | stable | stable     |
| Time to black ppt           | 16     | 48     | stable | stable | stable | D      | stable | stable     |

In view of the foregoing plating tests employing in the standard test plating bath sodium "Aerofloat" as the stabilizing agent, it will be observed that stabilization is obtained from 5-20 p. p. m. with an increased plating rate at the latter concentration.

In a series of these plating tests employing the standard test plating bath containing sodium "Aerofloat B" as the stabilizing agent, the following results were obtained:

Stability tests—60 minutes

| p. p. m. Sodium "Aerofloat B" | 1      | 5      | 10     | 20     | 30     | 50     | 300        |
|-------------------------------|--------|--------|--------|--------|--------|--------|------------|
| Wt. gain, gms                 | 0.1386 | 0.1459 | 0.1454 | 0.1502 | 0.0020 | D      | no plating |
| Sample appearance             | B-S    | BB-S   | BB-S   | BB-S   | stable | D      | stable     |
| Time to black ppt             | 33     | stable | stable | stable | D      | stable | stable     |

In view of the foregoing plating tests employing in the standard test plating bath sodium "Aerofloat B" as the stabilizing agent, it will be observed that stabilization is

75 range from about 1.0 to 10.0 p. p. m.

obtained from 5.0 to 20.0 p. p. m., with a somewhat increased plating rate in the latter concentration.

In a series of these plating tests employing the standard test plating bath containing thiomalic acid as the stabilizing agent, the following results were obtained:

(a) Rate tests—10 minutes

| p. p. m. thiomalic acid       | 0.5    | 1      | 5      | 10     | 50     |
|-------------------------------|--------|--------|--------|--------|--------|
| Wt. gain, gms                 | 0.0768 | 0.0900 | 0.0903 | 0.0928 | 0.0040 |
| Plating rate, $R \times 10^4$ | 3.84   | 4.50   | 4.51   | 4.60   | 0.02   |
| Sample appearance             | D-S    | B-S    | B-S    | B-S    | D-R    |
| Time to black ppt             | 5      | 10     | none   | none   | none   |

(b) Stability tests—60 minutes

| p. p. m. thiomalic acid | 0.5    | 1      | 5      | 10     | 50     |
|-------------------------|--------|--------|--------|--------|--------|
| Wt. gain, gms           | 0.1335 | 0.1415 | 0.1480 | 0.1446 | 0.0040 |
| Sample appearance       | D-SR   | B-S    | B-S    | B-S    | D-R    |
| Time to black ppt       | 5      | stable | stable | stable | stable |

In view of the foregoing plating tests employing in the standard test plating bath thiomalic acid as the stabilizing agent, it will be observed that stabilization is obtained between 1.0 and 10.0 p. p. m.

In a series of these plating tests employing the standard test plating bath containing thiocarbanilide as the stabilizing agent the following results were obtained:

Stability tests—60 minutes

| p. p. m. thiocarbanilide | 1      | 5      | 10     | 50         |
|--------------------------|--------|--------|--------|------------|
| Wt. gains, gms           | 0.1436 | 0.1456 | 0.1313 | no plating |
| Sample appearance        | B-S    | BB-S   | BB-S   | stable     |
| Time to black ppt        | 30     | stable | stable | stable     |

In these plating tests since thiocarbanilide is not water-soluble, it was first dissolved in ethylene glycol and then introduced into the standard test plating baths, whereby it was observed that thiocarbanilide stabilizes at 5.0 p. p. m. and above, plating being inhibited at 50.0 p. p. m.

In a series of these plating tests employing a standard test plating bath containing thiourea as a stabilizing agent, the following results were obtained:

Stability tests—60 minutes

| p. p. m. thiourea | 1      | 5      | 10     | 50         |
|-------------------|--------|--------|--------|------------|
| Wt. gain, gms     | 0.1402 | 0.1402 | 0.1340 | no plating |
| Sample appear     | BB-S   | BB-S   | BB-S   | stable     |
| Time to black ppt | stable | stable | stable | stable     |

In view of the foregoing plating tests employing in the standard test plating bath sodium "Aerofloat B" as the stabilizing agent, it will be observed that stabilization is

75 range from about 1.0 to 10.0 p. p. m.

Again it is pointed out that when the nickel cation concentration in the plating bath is increased, the amount of stabilizing agent that must be added thereto must be disproportionately increased as indicated by the plating tests appearing below utilizing the special test plating bath and plating procedure previously described.

In a series of these plating tests employing the special test plating bath containing sodium "Aerofloat" as the stabilizing agent, the following results were obtained:

(a) *Rate tests—10 minutes*

| p. p. m. sodium "Aerofloat"    | 1      | 5      | 10     | 15     | 20     |
|--------------------------------|--------|--------|--------|--------|--------|
| Wt. gain, gms.                 | 0.1309 | 0.1360 | 0.1361 | 0.1311 | 0.1212 |
| Plating rate RX10 <sup>4</sup> | 6.55   | 6.80   | 6.81   | 6.56   | 6.06   |
| Sample appearance              | BB-R   | BB-S   | BB-S   | BB-S   | BB-S   |
| Time to black ppt.             | 5      | none   | none   | none   | none   |

(b) *Stability tests—60 minutes*

| p. p. m. Sodium "Aerofloat" | 1      | 5      | 10     | 15     | 20     |
|-----------------------------|--------|--------|--------|--------|--------|
| Wt. gain, gms.              | 0.2020 | 0.2429 | 0.2511 | 0.2313 | 0.2302 |
| Sample appearance           | BB-R   | BB-R   | BB-S   | BB-S   | BB-S   |
| Time to black ppt.          | 5      | 20     | 40     | 58     | stable |

By comparison of the plating tests respectively involving the standard test plating bath and the special test plating bath, it will be observed that as little as 5.0 p. p. m. of sodium "Aerofloat" is effective to produce stabilization in the standard test plating bath, whereas 20.0 p. p. m. of sodium "Aerofloat" is required to effect stabilization in the special test plating bath. However, in the plating tests employing the special test plating bath, the plating rate is substantially increased and the sample appearance is brighter.

While the effective minimum amounts of the different ones of these organic stabilizing agents to achieve stabilization are a function of nickel cation concentration in the plating baths, as explained above, they are otherwise independent of the particular compositions of the plating baths with reference to other constituents. This is probably due to the fact that they do not form complexes with such constituents as malic acid, lactic acid, amino-acetic acid, etc. Thus the stabilizing agents of the organic type possess this advantage with respect to the stabilizing agents of the inorganic type, previously described. Moreover, when the stabilizing agents of the organic type are used in proper amounts, they do not decrease the plating rate over wide ranges, and they tend to increase substantially sample brightness; and moreover, they do not appear to have any adverse action on the adhesion of the nickel plating upon the base metal.

Furthermore, due to the exceedingly small amount of sulfide ion controller required in a plating bath, it is immaterial from an economic standpoint which one among those described above is selected and in what quantity it is used within the individual operating range thereof, providing that the plating rate is not decreased.

It will be understood that the stabilizing agents described are particularly well-suited for use in continuous nickel plating processes involving regeneration of the ingredients of the character disclosed in the Talmey and Crehan application.

It should be noted that analytic methods for the "exact" determination of trace quantities of ingredients of the order of magnitude herein employed (for example, sulfide ion controller in parts per 1,000,000,000 parts of the plating bath) are not now available in the art; however, these trace quantities as set forth were determined by carefully eliminating all possible sources of sulfide and other trace ions from the plating bath, and then by adding known quantities thereof to the bath. Accordingly, it will be appreciated that the trace quantities given are approximate, but are readily understandable by those

skilled in the art, as levels above the maximum obtainable purity of ingredients employed in the formation of the plating bath.

In view of the foregoing, it is apparent that there has been provided an improved process of chemical nickel plating of catalytic materials employing baths of the nickel cation-hypophosphite anion type containing stabilizing agents, as well as improved baths therefor. Further, it will be understood that great advantages are obtained by the utilization of the present process, particularly in continuous nickel plating operations, since such processes frequently involve exceedingly large volumes of the nickel plating bath that must be stabilized.

While there has been described what is at present considered to be the preferred embodiment of the invention, it will be understood that various modifications may be made therein, and it is intended to cover in the appended claims all such modifications as fall within the true spirit and scope of the invention.

20. *What is claimed is:*

1. The process of chemically plating with nickel a body essentially comprising an element selected from the group consisting of iron, cobalt, nickel, aluminum, copper, silver, gold, palladium and platinum, which comprises contacting said body with an aqueous bath consisting essentially of nickel ions and hypophosphite ions and also containing sulfide ions and a sulfide ion controller, both said sulfide ions and said sulfide ion controller being present in solution in said bath only in controlled trace amounts that together are not greater than about 200 parts per 1,000,000 parts of said bath by weight so as not substantially to reduce the plating rate of said bath, said sulfide ion controller forming with said sulfide ions a thio-compound that is both stable and substantially insoluble in said bath so as to maintain the dissociated sulfide ion concentration in said bath of the order of magnitude of 1 part per 100,000,000 parts of said bath by weight in order to inhibit random decomposition of said bath.

40. 2. The process of chemically plating with nickel a body essentially comprising an element selected from the group consisting of iron, cobalt, nickel, aluminum, copper, silver, gold, palladium and platinum, which comprises contacting said body with a hot aqueous bath consisting essentially of nickel ions and hypophosphite ions and also containing sulfide ions and a sulfide ion controller, the temperature of said bath being above 90° C. and the pH of said bath being in the range 3.0 to 8.5, both said sulfide ions and said sulfide ion controller being present in solution in said bath only in controlled trace amounts that together are not greater than about 200 parts per 1,000,000 parts of said bath by weight so as not substantially to reduce the plating rate of said bath, said sulfide ion controller forming with said sulfide ions a thio-compound that is both stable and substantially insoluble in said bath so as to maintain the dissociated sulfide ion concentration in said bath of the order of magnitude of 1 part per 100,000,000 parts of said bath by weight in order to inhibit random decomposition of said bath.

60. 3. The process of chemically plating with nickel a body essentially comprising an element selected from the group consisting of iron, cobalt, nickel, aluminum, copper, silver, gold, palladium and platinum, which comprises contacting said body throughout a given time interval with an aqueous bath consisting essentially of nickel ions and hypophosphite ions and also containing sulfide ions and a sulfide ion controller, both said sulfide ions and said sulfide ion controller being present in solution in said bath only in controlled trace amounts that together are not greater than about 200 parts per 1,000,000 parts of said bath by weight so as not substantially to reduce the plating rate of said bath, said sulfide ion controller forming with said sulfide ions a thio-compound that is both stable and substantially insoluble in said bath

21

so as to maintain the dissociated sulfide ion concentration in said bath of the order of magnitude of 1 part per 100,000,000 parts of said bath by weight in order to inhibit random decomposition of said bath, maintaining the temperature of said bath above 90° C. throughout said given time interval, maintaining the pH of said bath in the range 3.0 to 8.5 throughout said given time interval, and adding to said bath during said given time interval trace quantities of both said sulfide ions and said sulfide ion controller so as to maintain said controlled trace amounts thereof in said bath throughout said given time interval.

4. The process of chemically plating with nickel a body essentially comprising an element selected from the group consisting of iron, cobalt, nickel, aluminum, copper, silver, gold, palladium and platinum, which comprises contacting said body with an aqueous bath consisting essentially of nickel ions and hypophosphite ions and an additive consisting of a thio-compound having a dipolar molecular structure including a dissociable cation and a hydrophobic anion forming with said element a compound insoluble in said bath, said additive being present in solution in said bath only in a controlled trace amount not greater than about 200 parts per 1,000,000 parts of said bath by weight so as not substantially to reduce the plating rate of said bath and so as to inhibit random decomposition of said bath.

5. The process of chemically plating with nickel a solid body essentially comprising an element selected from the group consisting of iron, cobalt, nickel, aluminum, copper, silver, gold, palladium and platinum, which comprises contacting said body with an aqueous bath consisting essentially of nickel iron and hypophosphite ions and an additive consisting of a thio-compound that forms an oriented hydrophobic film on said body, said additive being present in solution in said bath only in a controlled trace amount not greater than about 200 parts per 1,000,000 parts of said bath by weight so as not substantially to reduce the plating rate of said bath and so as to inhibit random decomposition of said bath.

6. The process set forth in claim 5, wherein said additive consists essentially of a sulfhydric compound.

7. The process of chemically plating with nickel a body essentially comprising an element selected from the group consisting of iron, cobalt, nickel, aluminum, copper, silver, gold, palladium and platinum, which comprises contacting said body with an aqueous bath consisting essentially of nickel ions and hypophosphite ions, said bath also containing a thio-compound that is both non-catalytic for the oxidation of hypophosphite and stable in said bath, said thio-compound being present in solution in said bath only in a controlled trace amount not greater than about 200 parts per 1,000,000 parts of said bath by weight so as not substantially to reduce the plating rate of said bath and so as to maintain the dissociated sulfide ion concentration in said bath only in a controlled trace amount of the order of magnitude of 1 parts per 100,000,000 parts of said bath by weight in order to inhibit random decomposition of said bath.

8. The process set forth in claim 7, wherein said thio-compound consists essentially of an organic thio-compound.

9. The process set forth in claim 7, wherein said thiocompound consists essentially of an xanthate.

10. The process set forth in claim 7, wherein said thio-compound consists essentially of a thio-phosphate.

11. The process set forth in claim 10, wherein said thio-phosphate has the general structural formula:



where R is a radical selected from the group consisting of alkyl and aryl, and X is an ion selected from the

22

group consisting of hydrogen, alkali metal and ammonium.

12. The process of chemically plating with nickel a body essentially comprising an element selected from the group consisting of iron, cobalt, nickel, aluminum, copper, silver, gold, palladium and platinum, which comprises contacting said body with an aqueous bath consisting essentially of nickel ions and hypophosphite ions, said bath also containing sulfide ions and ions of a heavy metal that is non-catalytic for the oxidation of hypophosphite and that forms with said sulfide ions a thio-compound that is both stable and substantially insoluble in said bath, said thio-compound being present in solution in said bath only in a controlled trace amount not greater than about 200 parts per 1,000,000 parts of said bath by weight so as not substantially to reduce the plating rate of said bath and so as to maintain the dissociated sulfide ion concentration in said bath only in a controlled trace amount of the order of magnitude of 1 part per 100,000,000 parts of said bath by weight in order to inhibit random decomposition of said bath.

13. The process of chemically plating with nickel a body essentially comprising an element selected from the group consisting of iron, cobalt, nickel, aluminum, copper, silver, gold, palladium and platinum, which comprises contacting said body with an aqueous bath consisting essentially of nickel ions and hypophosphite ions, said bath also containing a sulfide of a metal selected from the group consisting of lead, tellurium and tin, said metal sulfide being present in solution in said bath only in a controlled trace amount not greater than about 50 parts per 1,000,000 parts of said bath by weight so as not substantially to reduce the plating rate of said bath and so as to maintain the dissociated sulfide ion concentration in said bath only in a controlled trace amount of the order of magnitude of 1 part per 100,000,000 parts of said bath by weight in order to inhibit random decomposition of said bath.

14. The process of chemically plating with nickel a body essentially comprising an element selected from the group consisting of iron, cobalt, nickel, aluminum, copper, silver, gold, palladium and platinum, which comprises contacting said body with an aqueous bath consisting essentially of nickel ions and hypophosphite ions, said bath also containing lead sulfide, said lead sulfide being present in solution in said bath only in a controlled trace amount not greater than about 5 parts per 1,000,000 parts of said bath by weight so as not substantially to reduce the plating rate of said bath and so as to maintain the dissociated sulfide ion concentration in said bath only in a controlled trace amount of the order of 1 part per 100,000,000 parts of said bath by weight in order to inhibit random decomposition of said bath.

15. The process of chemically plating with nickel a body essentially comprising an element selected from the group consisting of iron, cobalt, nickel, aluminum, copper, silver, gold, palladium and platinum, which comprises contacting said body with an aqueous bath consisting essentially of nickel ions and hypophosphite ions, said bath also containing sulfide ions and ions of lead, said sulfide ions and ions of lead being present in solution in said bath only in controlled trace amounts that together are not greater than about 5 parts per 1,000,000 parts of said bath by weight so as not substantially to reduce the plating rate of said bath and so as to maintain the dissociated sulfide ion concentration in said bath in a controlled trace amount of the order of magnitude of 1 part per 100,000,000 parts of said bath by weight in order to inhibit random decomposition of said bath.

16. The process of chemically plating with nickel a body essentially comprising an element selected from the group consisting of iron, cobalt, nickel, aluminum, copper, silver, gold, palladium and platinum, which comprises contacting said body with an aqueous bath consisting essentially of nickel ions and hypophosphite ions, said

bath also containing sulfide ions and ions of tellurium, said sulfide ions and ions of tellurium being present in solution in said bath only in controlled trace amounts that together are not greater than about 200 parts per 1,000,000 parts of said bath by weight so as not substantially to reduce the plating rate of said bath and so as to maintain the dissociated sulfide ion concentration in said bath only in a controlled trace amount of the order of magnitude of 1 part per 100,000,000 parts of said bath by weight in order to inhibit random decomposition of said bath.

17. The process of chemically plating with nickel a body essentially comprising an element selected from the group consisting of iron, cobalt, nickel, aluminum, copper, silver, gold, palladium and platinum, which comprises contacting said body with an aqueous bath consisting essentially of nickel ions and hypophosphite ions, said bath also containing sulfide ions and ions of tin, said sulfide ions and ions of tin being present in solution in said bath only in controlled trace amounts that together are not greater than about 125 parts per 1,000,000 parts of said bath by weight so as not substantially to reduce the plating rate of said bath and so as to maintain the dissociated sulfide ion concentration in said bath only in a controlled trace amount of the order of magnitude of 1 part per 100,000,000 parts of said bath by weight in order to inhibit random decomposition of said bath.

18. The process of chemically plating with nickel a body essentially comprising an element selected from the group consisting of iron, cobalt, nickel, aluminum, copper, silver, gold, palladium and platinum, which comprises contacting said body throughout a time interval with an aqueous bath consisting essentially of nickel ions and hypophosphite ions, said bath also containing lead sulfide, said lead sulfide being present in solution in said bath only in a controlled trace amount in the approximate range .5 to 5 parts per 1,000,000 parts of said bath by weight so as not substantially to reduce the plating rate of said bath and so as to maintain the dissociated sulfide ion concentration in said bath only in a controlled trace amount of the order of 1 part per 100,000,000 parts of said bath by weight in order to inhibit random decomposition of said bath, and adding to said bath during said time interval trace quantities of both sulfide ions and lead ions so as to maintain said controlled trace amount of lead sulfide present in solution in said bath in said range set forth.

19. The process of chemically plating with nickel a body essentially comprising an element selected from the group consisting of iron, cobalt, nickel, aluminum, copper, silver, gold, palladium and platinum, which comprises contacting said body with a hot aqueous bath consisting essentially of nickel ions and hypophosphite ions and also containing  $S^{''}$  anions and  $Pb^{+}$  cations in controlled trace amounts that together are not greater than about 10 parts per 1,000,000 parts of said bath by weight so as not substantially to reduce the plating rate of said bath, the temperature of said bath being above 90° C. and the pH of said bath being in the range 3.0 to 7.0, the  $Pb^{+}$  cation concentration in said bath being in the approximate range 0.5 to 5.0 parts per 1,000,000 parts of said bath by weight so as to maintain the dissociated  $S^{''}$  anion concentration in said bath of the order of magnitude of 1 part per 100,000,000 parts of said bath by weight in order to inhibit random decomposition of said bath.

20. The process of chemically plating with nickel a body essentially comprising an element selected from the group consisting of iron, cobalt, nickel, aluminum, copper, silver, gold, palladium and platinum, which comprises contacting said body with an aqueous bath comprising nickel ions and hypophosphite ions, said bath also containing some sulfur and a trace of lead in solution therein in order to inhibit random decomposition thereof without substantial reduction of the plating rate thereof,

said trace of lead in solution in said bath being in an amount by weight of at least  $\frac{1}{2}$  part but not in excess of 5 parts per 1,000,000 parts of said bath.

5 21. The process of chemically plating with nickel a body essentially comprising an element selected from the group consisting of iron, cobalt, nickel, aluminum, copper, silver, gold, palladium and platinum, which comprises contacting said body with an aqueous bath comprising nickel ions and hypophosphite ions, said bath 10 also containing some sulfur and a trace of lead in solution therein in order to inhibit random decomposition thereof, said trace of lead in solution in said bath being in an amount by weight of about 2 parts per 1,000,000 parts of said bath.

20 22. A bath for the chemical plating of a catalytic material with nickel consisting essentially of an aqueous solution of a nickel salt and a hypophosphite and an additive consisting of a thio-compound that forms an oriented hydrophobic film on said material, said additive being present in solution in said bath only in a controlled trace amount not greater than about 200 parts per 1,000,000 parts of said bath by weight so as not substantially to reduce the plating rate of said bath and so as to inhibit random decomposition of said bath.

25 23. The bath set forth in claim 22, wherein said additive consists essentially of a sulfhydryl compound.

30 24. A bath for the chemical plating with nickel of a catalytic material consisting essentially of an aqueous solution of a nickel salt and a hypophosphite, said bath also containing a thio-compound that is both non-catalytic for the oxidation of hypophosphite and stable in said bath, said thio-compound being present in solution in said bath only in a controlled trace amount in the approximate range 0.05 to 200 parts per 1,000,000 parts of said bath by weight so as not substantially to reduce the plating rate of said bath and so as to maintain the dissociated sulfide ion concentration in said bath only in a controlled trace amount of the order of magnitude of 1 part per 100,000,000 parts of said bath by weight in order to inhibit random decomposition of said bath.

35 25. A bath for the chemical plating with nickel of a catalytic material consisting essentially of an aqueous solution of a nickel salt and a hypophosphite, said bath also containing sulfide ions and ions of lead, said ions named being present in solution in said bath only in controlled trace amounts that together are not greater than about 5 parts per 1,000,000 parts of said bath by weight so as not substantially to reduce the plating rate of said bath and so as to maintain the dissociated sulfide ion concentration in said bath in a controlled trace amount of the order of magnitude of 1 part per 100,000,000 parts of said bath by weight in order to inhibit random decomposition of said bath.

40 26. A bath for the chemical plating with nickel of a catalytic material comprising an aqueous solution of a nickel salt and a hypophosphite, said bath also containing some sulfur and a trace of lead in solution therein in order to inhibit random decomposition thereof without substantial reduction of the plating rate thereof, said trace of lead in solution in said bath being in an amount by weight of at least  $\frac{1}{2}$  part but not in excess of 5 parts per 1,000,000 parts of said bath.

45 27. A bath for the chemical plating with nickel of a catalytic material comprising an aqueous solution of a nickel salt and a hypophosphite, said bath also containing some sulfur and a trace of lead in solution therein in order to inhibit random decomposition thereof without substantial reduction of the plating rate thereof, said trace of lead in solution in said bath being in an amount by weight of about 2 parts per 1,000,000 parts of said bath.

50 References Cited in the file of this patent

UNITED STATES PATENTS

75 2,532,283 Brenner ----- Dec. 5, 1950